

Nov. 23, 1954

V. V. DE OLLOQUI ET AL.

**2,695,256**

## LIGHTWEIGHT BATHTUB AND PRODUCTION THEREOF

Filed Nov. 12, 1952

-F1 Q-1

2 Sheets-Sheet 1



## Inventors

Valentine V. De Olloqui  
Carl A. Strand &  
Carroll H. Van Hartesveldt

Carroll H. Van Hartesveldt  
By Will Sherman, Moran, Good & Simpson AT&T 45

Nov. 23, 1954

V. V. DE OLLOQUI ET AL

2,695,256

LIGHTWEIGHT BATHTUB AND PRODUCTION THEREOF

Filed Nov. 12, 1952

2 Sheets-Sheet 2

FIG-6



FIG-8



FIG-7

INVENTORS  
Valentine V. De Olloqui  
Carl A. Strand &  
Carroll H. Van Hartesveldt

Tele. Sherman, Meconi, Grass, Simpson, ETC.

# United States Patent Office

2,695,256

Patented Nov. 23, 1954

1

2,695,256

## LIGHTWEIGHT BATHTUB AND PRODUCTION THEREOF

Valentine V. de Olioqui, Cleveland Heights, Ohio, and Carl A. Strand and Carroll H. Van Hartesveldt, Birmingham, Mich., assignors to Carl A. Strand, doing business as Strand-Plax Building Products Co., Birmingham, Mich.

Application November 12, 1952, Serial No. 319,992

11 Claims. (Cl. 154—83)

This invention relates to light weight bathtubs or the like receptacles and the production thereof, and more particularly, to a specific glass fiber-polyester laminated bathtub and the production thereof.

As is well known, the ordinary bathtub is a very heavy cast iron receptacle, which is expensive to produce and also to install. In addition, such cast iron bathtubs are extremely difficult to handle during shipment and installation because of their very great weight. This excessive weight also prevents or substantially limits the use of such bathtubs in living quarters wherein weight of fixtures is a distinct disadvantage, for example, in light-weight cabins, temporary houses, certain forms of prefabricated dwellings, and particularly in automobile trailer houses.

The substitution of other materials for the enamel-coated cast iron bathtub has, however, provided a problem which heretofore has gone unsolved, notwithstanding the very great need for bathtubs as units of substantially lighter weight. The enamel coating, which is employed for decorative purposes as well as for the purpose of simplifying the cleaning of the bathtub, is characterized by extreme brittleness typical of ceramic materials; and such enamel coating must be supported by an extremely strong and inflexible structure or shell in order to prevent fracture thereof during ordinary wear and tear, and particularly in response to sharp impact. The use of cast iron in the formation of such a shell has, therefore, been considered a necessity, heretofore.

The instant invention provides a unique solution to this heretofore unsolved problem by providing a substantially improved "enamel-like" coating material, which may be substantially integrally formed with a specially built light weight bathtub shell. The instant body of the shell provides the structural strength, and in addition a certain amount of resilience, and the instant coating provides the necessary high-gloss clean white finish which is substantially integral with the shell and which is, in and of itself, sufficiently resilient to resist (in combination with the shell) the ordinary strains and impacts suffered by a bathtub during ordinary wear and tear.

It is, therefore, an important object of the instant invention to provide an improved light weight bathtub and an improved method of producing the same.

A further object of the instant invention is to provide, as an improved article of manufacture, a light weight bathtub having a suitably formed integral body of a laminate composed of one part of glass fibers embedded in two parts of normally rigid thermoset unsaturated polyester laminating resin, and having a smooth-surfaced glossy coating integrally formed upon the body, said coating consisting essentially of one part of pigment-size filler embedded in two parts of a thermoset unsaturated polyester mixture of equal parts of normally rigid and normally flexible polyesters.

It is another object of the instant invention to provide an improved light weight bathtub having a suitably formed integral body of a laminate composed of one part of glass fibers embedded in one to three parts of normally rigid thermoset unsaturated polyester laminating resin, and having a smooth-surfaced coating integrally formed upon the body, said coating consisting essentially of 10-30% titanium dioxide pigment, 5-15% finely ground amorphous silica filler and 60-70% of a cured polyester mixture of 50-60% unsaturated polyester and 40-50% saturated polyester.

2

Still a further object of the instant invention is to provide an improved method of forming a light weight bathtub that comprises applying a 0.01-0.02 inch coating to a mirror-finish convex surface of the contour of the inside of the bathtub, said coating being composed of 10-30% titanium dioxide pigment, 5-15% finely ground amorphous silica filler, a catalyst mixture of a metal drier and a ketone peroxide, and 60-70% of a polymerizable polyester mixture of 50-60% unsaturated polyester and 40-50% saturated polyester; then covering the coating with a layer of glass fibers impregnated with twice their weight of polymerizable unsaturated polyester containing a metal drier-ketone peroxide catalyst mixture; and finally applying heat and pressure to the coating and impregnated glass fibers to cure the polyesters therein.

It is yet another object of the instant invention to provide an improved, light weight, shock-resistant, inexpensive, easily handled bathtub that has substantially better heat-insulating properties than cast iron, that is more easily installed than a cast iron bathtub, and that has a highly scratch-resistant smooth glossy finish thereon, and an improved method of making such bathtub.

Other and further objects, features and advantages of the present invention will become apparent to those skilled in the art from the following detailed description of preferred embodiment thereof, and the attached drawings which form a part of this specification.

On the drawings:

Figure 1 is a side elevational view of a light weight bathtub embodying the instant invention, shown in the environment of its installation;

Figure 2 is a sectional elevational view taken substantially along the line II—II of Figure 1;

Figure 3 is a sectional elevational enlarged detail view showing the cooperation between the top edge of one side of the tub and a front panel supporting member;

Figure 4 is an elevational sectional view of a suitable mold having a coating applied thereto during an initial step in the method of preparing the instant light weight bathtub;

Figure 5 is a top plan view of a glass mat employed in one of the production methods embodying the instant invention for producing the light weight bathtub;

Figure 6 is a sectional elevational view of a suitable low pressure laminating mold assembly that is used in carrying out the production method wherein the glass fiber mat of Figure 5 is used;

Figure 7 is essentially a diagrammatical view showing how a pre-formed impregnated glass fiber shell may be preferred for use in a second production method embodying the instant invention; and

Figure 8 is essentially an exploded sectional elevational view showing the mold parts and elements employed in the production method employing the pre-formed shell prepared as shown in Figure 7.

As shown on the drawings:

As shown in Figures 1 and 2, the instant light weight bathtub, indicated generally by the reference numeral 10, comprises a suitably formed glass fiber-polyester laminated bathtub shell 11 having upwardly extending front 12 and back 13 side walls, and left 14 and right 15 end walls. The back side wall 13 extends upwardly and flares outwardly at 13a to engage and be supported by the bathroom wall W. As will be seen, the extreme top of the back wall 13 has an upwardly extending rib 13b which interlocks with suitably positioned tile T mounted on the bathroom wall W in the usual manner. The tile on back wall are shown essentially diagrammatically only in Figure 2 to avoid undue confusion in the drawings.

The end walls 14 and 15 like the back wall 13 extend upwardly and outwardly to define ridges 14b and 15b, respectively, which engage the walls W, W and coact therewith in substantially the same manner that the back wall 13 engages and is supported by the bathroom wall.

The remaining wall, the front wall 12, extends upwardly and near the top thereof at 12a is turned outwardly and down, so as to define in cross section at the top 12a a curved arch, as is best shown in Figure 3. The arch 12a terminates at its outer extremity 12b with a substantially downwardly directed rib portion. This end portion 12b seats firmly in the front groove 16a of

an S-shaped elongated metal strip 16 which extends the full longitudinal direction of the shell 11 and arcuate front wall top 12a. The rear groove 16b of the S-shaped strip 16 securely seats the rounded top edge of a supporting panel 17 which extends vertically upwardly from the floor F. The panel 17 is rigidly secured to the floor F, for example, by means of a screw and sprocket assembly 18, and the panel 17 extends the full longitudinal dimension of the shell 11 and upwardly to substantially the height of the arcuate top 12a of the front wall 12. The panel 17 is made of suitably strong structural wood, plywood, heavy-weight laminate or the like material, which is capable of withstanding very substantial downward pressure and which is sufficiently rigidly secured to the floor F to resist substantial lateral directed forces, so as to afford a certain amount of protection for the front wall 12. The front wall 12 is made of a suitably strong glass fiber-polyester laminate material that is capable of withstanding very substantial downwardly directed forces, and the front wall 12 and panel 17 (by virtue of its supporting engagement with the outer lip 12b of the front wall 12) cooperate to provide very substantial force-resisting support for the top arcuate portion 12a.

In this manner, the top arcuate portion 12a is capable of readily withstanding the ordinary wear and tear during use of the instant bathtub assembly 10, as is particularly capable of withstanding the weight of human beings leaning on or pulling against the arcuate portion 12a, while getting in and out of the bathtub 10. It will be appreciated that the panel 17 may be easily installed at the same time the bathtub 10 is installed and the panel 17 may be prefabricated of the desired weight and strength to carry out its particular function just described. It will also be appreciated that in the use and installation of the ordinary cast iron bathtub a structure generally similar to the instant shell structure 11 is employed with a depending wall member, also made of cast iron, which takes the place of the panel 17. In such an arrangement the depending wall member furnishes the sole support for substantially the entire weight of the cast iron tub, and the top edges of the other walls of the top shell tub, and the top edges of the other walls of the top shell tub, are suitably affixed to the bathroom walls.

The instant top shell 11 is, however, not supported entirely by the panel 17. In fact, because of its light weight and other advantageous features connected therewith, the overall shell 11 is too resilient in character to be supported by the panel 17 alone. It is also necessary to employ a suitable rack or supporting device 18 which is centrally positioned beneath the top shell 11.

As will be seen, the rack 18 consists of a plurality of longitudinally extending generally flat members 19, which are suitably mounted on the curved tops of laterally extending spaced beams 20, which are in turn tied together by tie rods or side boards 21. It will thus be seen that the rack 18 is suitably mounted on the floor level and extends upwardly to support the central portion of the shell bottom, which is itself a generally dish-shaped bottom that is sloped downwardly into the direction of the drain 22 and which becomes decreasingly bowed or dished in shape in the longitudinal direction toward the drain 22 (or the drain end 14 of the shell 11).

A particularly important aspect of the instant invention resides in the particular structural arrangement and composition combination employed in the bathtub shell 11, and the method of fabricating this shell 11. Actually, the shell 11 is composed of a body or structural portion 23 and an integral coating 24, as is best shown in Figure 6. In general, the bathtub shell 11 has a suitably formed integral body 23 of a laminate composed of one part of glass fibers embedded in from one to three parts of normally rigid thermoset unsaturated polyester laminating resin, and it has a smooth-surfaced glossy coating 24 integrally formed upon the body 23. The coating consists essentially of one part of pigment-size filler embedded in two parts of a thermoset unsaturated polyester mixture of equal parts of normally rigid and normally flexible polyester. It is believed, however, that certain of the critical aspects of the instant structure and composition will be thus appreciated from a study of the methods employed in preparing the instant bathtub shell 11.

In one method, which method will be referred to hereinafter as method A, certain steps of which are described or illustrated in connection with Figures 4, 5 and 6, the first step is that of applying the coating 24 to a suitably shaped generally concavo-convex mold form 25, whose

outer surface is shaped to conform with the inside surface of the desired bathtub shell 11. As will be appreciated, the mold form 25 curves outwardly and then sharply downwardly, such as at 25a, along three sides of the base of the mold form 25, in order to correspond to the general shape of the upstanding ridges 13b, 14b and 15b, hereinbefore described. On the remaining side of the base of the form 25, there is provided a generally arcuate side portion 25b which defines the outer surface of the arcuate portion 12a of the front wall 12. A suitable spacer support 26 is positioned around the bottom of the form 25 so as to level the same.

The first step in method A is that of applying the desired coating 24 to the outer surface of the mold form 25, as described. A particularly important feature of this process resides in the fact that the outer surface of the mold form 25 is mirror-finished. This is particularly important since it is desired to impart to the ultimately exposed base of the coating 24 a mirror-finished glossy appearance. The mold form 25 is usually coated with a small amount of wax or the like mold lubricant prior to the application of the coating composition 24. The coating composition 24 is then applied to the mold form 25 by means of a spraying unit 27, or by means of any other suitable coating applying devices or processes. Most preferably, the coating is sprayed upon the form 25, to apply a uniformly thick coating 24 having approximately 0.01-0.02 inch thickness. The consistency of the coating 24 is preferably such that the coating adheres at the location at which it is sprayed upon the form 25 and does not run or gather near the base of the form 25. In the event that the coating may have a tendency to run slightly, the form 25 may be heated slightly to cause at least a limited amount of preliminary curing to take place in the coating so that the same will adhere at a given location. Also, if a solvent or vehicle is employed to assist in applying the coating to the form 25, then it is usually desirable to heat the walls 25 in order to drive off the solvent and to leave the coating 24 in the desired thickness hereinbefore mentioned.

As previously indicated, the essential ingredients of the coating thus applied include about one part of pigment-size filler intimately admixed with about two parts of a fluid polymerizable unsaturated polyester mixture, which will be described in detail hereinafter. Most preferably, the pigment-size filler is made up of about one part of finely ground amorphous silica filler, or any other inorganic inert finely ground filler which preferably is white or substantially uncolored; and about two parts of titanium dioxide pigment, which has been found to be by far the most superior white pigment (and the use of other white pigments, although inferior in most instances, would not necessarily be contrary to the principles of this invention, for certain special uses). As will be appreciated, it is desired to obtain a mirror-finish high gloss type of coating herein and, accordingly, substantially fine, pigment-size filler materials as well as pigments must be used. Actually, the very substantial amount of titanium dioxide employed permits this ingredient to function both as a filler and as a pigment, and the titanium dioxide may be used in proportions within the range of about 10-30 weight percent of the coating mixture. The finely ground amorphous silica filler is employed principally to incorporate a sufficient amount of filler in the coating composition to impart the desired high viscosity thereto, as well as the necessary superior strength in the finally cured or hardened coating 24. The amount of such silica filler which may be used may be within the range of about 5-15 weight percent of the coating composition.

(As used herein the terms "parts" and "percent" mean parts and percent by weight, unless otherwise specified.) The remaining ingredient in the coating composition is the polymerizable unsaturated polyester mixture, with the necessary curing or accelerating catalysts incorporated therein. As previously indicated, in the most preferred coating composition about one part of the silica filler, and about two parts of titanium dioxide pigment are admixed with about six to seven parts of the unsaturated polyester mixture. Actually, however, the proportions may be as follows:

10-30% titanium dioxide

5-15% ground silica filler

60-70% polymerizable polyester mixture and the necessary catalyst mixture of ketone peroxide and metal drie

As will be appreciated, it is often desirable to include in trace amounts certain other tinting agents which assist in giving a richer white color to the coating, such agents including for example iron oxide pigment. Some of the metal driers which are employed in the catalyst also may act as tinting agents to limited extents; and the selection of such tinting agents is well within the skill of those familiar with the pigment art.

In connection with the polymerizable polyester mixture, it is known generally that the polyester resins may be prepared by esterification-condensation of a polybasic acid (preferably a dicarboxylic acid) and a polyhydroxy alcohol (preferably a dihydric alcohol), in the substantial absence of addition polymerization-inducing conditions. As a typical member of the thermosetting polymerizable polyester which may be cured to form a normally rigid thermoset resin, the polyester resulting from such condensation of maleic acid (or anhydride) with ethylene glycol is mentioned. This polyester is generally referred to in the art as "ethylene glycol-maleate," or in the event that a slight amount (i. e. about 10%) of propylene glycol and of phthalic anhydride have also been employed, as is customary in the preparation of laminating resins, the resin is called "ethylene glycol-propylene glycol-phthalate-maleate" and so forth. In general, this polyester is an unsaturated dihydric alcohol-dicarboxylic acid (the unsaturation being furnished by the maleyl radicals therein, which are at least about 60-75 mol percent of the acyl radicals present, the remainder being phthalyl radicals preferably). Often such laminating resins contain a small proportion of a suitably co-polymerizable unsaturated monomer such as styrene or diallyl phthalate in order to assist in the cross-linking process during polymerization; but the general characteristics of these "structural" or "laminating" unsaturated polyester resins are those of the true polyester resin system. In other words, the resin is first obtained by the formation of long polyester chain-like molecules which are formed by condensation in the absence of addition polymerization and result in molecular chains having a plurality of unsaturated maleyl radicals therein. When such resins are cured, by addition polymerization, the maleyl radicals form cross-links between the chains thus changing the polymer from "linear" to "three-dimensional" and resulting in a rigid thermoset resin.

It has been found, however, that a flexible, substantially thermoset polyester may also be obtained. In this case the polymerizable polyester is substantially saturated instead of being substantially unsaturated, as just described. Such a resin may be an ethylene glycol-phthalate having perhaps 1-10 mol percent and preferably about 2-5 mol percent of the acid radicals as maleyl radicals and the remainder as phthalyl radicals. The "flexible" and the "structural" (or substantially rigid) polyester resins are both commercially available, and are so designated in industry.

In the instant coating composition, it has already been mentioned that about equal proportions of each such resins may be used. Hereinafter we shall refer to the structural as a "polymerizable unsaturated polyester" which may be thermoset to form a "normally rigid polyester"; and the flexible as a "saturated polyester" which may be cured or set to form a "normally flexible polyester." In admixture, in the coating composition, it has been found that good results are obtained using about 30-50% saturated polyester and about 70-50% unsaturated polyester, and most preferably 40-50% saturated and 60-50% unsaturated polyester.

The catalyst mixture here used is preferably a mixture of peroxide paste, containing equal parts of an organic peroxide and tricresyl phosphate dispersing agent, and a metal drier. The peroxide paste : metal drier ratio is about 3-2 : 2-1. Most preferably the peroxide employed is a ketone peroxide such as cyclohexanone peroxide which effects a minimum of discoloration during its acceleration of the addition polymerization; and the most active drier preferably used is a cobalt drier, cobalt naphthenate or cobalt maleate. The drier improves the hardness and final cure of the polyester at the air-exposed surfaces thereof. In the instant composition, most preferably about 3% of paste and 2% of the drier is used.

After the thin (i. e. about 0.01-0.02 inch thick) coating 24 has been applied to the mirror-finished mold form 25, the next step is that of preparing the glass fiber-resin

body 23. In accordance with the procedure of method A, a plurality (preferably only two) glass fiber mats, such as the mat 28 of Figure 5, are cut so as to fold over the coated surface of the mold form 25 and to be substantially co-extensive therewith. The glass fiber mats 28 are thus formed in the shape of a large rectangle with cuts taken out of the four corners, as shown in Figure 5. Such glass fiber mats are commercially available in relatively thin form comprising a great plurality of glass fibers or glass fiber strands heterogeneously arranged in the form of a sheet, but sufficiently entangled with each other to form a generally cohesive or unitary sheet, which may be cut and otherwise handled as a sheet of fabric in many respects. Such glass fiber mats 28 may be pre-treated with polyester resin, or they may be placed upon the coated mold form 25 and then have the necessary laminating polyester resin poured thereover so as to completely impregnate the mats 28. The amount of such laminating resin ordinarily required to accomplish this may range from about 1 to about 3 times the weight of the mats 28, and is most preferably about twice the weight of the mat. The polyester laminating resin employed for this purpose is the structural or unsaturated laminating resin hereinbefore described. As previously mentioned, the structural or unsaturated polyester resin is a resin which normally forms a rigid thermoset polyester resin upon additional polymerization thereof. It is known that such polyester when hardened is very rigid and perhaps even slightly brittle, if no filler is present therein. The impregnation of finely ground filler particles, or pigment-size particles, does not subtract substantially from the generally rigid nature of such polyester, so in the case of the instant coating composition we have added the flexible polyester in order to effectively obtain a coating which has the desired degree of resiliency or flexibility. It has also been found, however, that if certain fillers, namely, an elongated thin rod-like filler material such as glass fibers of substantial lengths, for example, at least an inch or two and preferably of substantially the entire length of the glass fiber mats, is present in a thermoset normally rigid polyester, a certain limited amount of true resiliency is imparted to the body. This resiliency is based upon a uniquely superior adherence between the glass fibers and the hardened polyester, as well as a certain amount of interference with the polyester cross linking, which results from the presence of the rather substantial amount of glass fibers in the body. Accordingly, it is not necessary to incorporate a certain amount of the flexible polyester in the binding agent for the glass fiber mat portion of the instant shell 11, although in certain special situations it may be possible to employ about 5-10% flexible polyester in order to obtain certain special properties, as in situations in which a relatively higher proportion of resin to glass fiber is employed. Most preferably, the laminating resin composition with which the glass fiber mats are impregnated consists essentially of about 97% of the unsaturated polymerizable polyester laminating resin, about 2% of the peroxide paste hereinbefore described and about 1% of a metallic drier.

After the suitably impregnated glass fiber mats have been properly positioned upon the coated mold form 25, the next step in method A involves, as shown in Figure 6, the complete envelopment of the stacked assembly in a flexible plastic molding bag 29. The bag 29 is a substantially air-tight molding bag of the type used for the formation of low pressure laminates, and after the bag has been closed upon the assembly, a pump 30, or the like evacuating device is used to exhaust all the air from inside the bag 29 so as to cause the bag to be stretchingly urged against the outside surface of the body 23, and to urge the body 23 into close engagement with the coating 24. The resulting body 23 (plus coating 24) thus has a thickness of approximately 0.06-0.08 inch, and the coating has the thickness of about 0.01-0.02 inch. Most preferably, the total thickness of the coating and body combined is approximately 0.08 inch.

The entire assembly with the bag 29 clamped thereagainst is then heated to the necessary curing temperature, so as to effect the required addition polymerization of the polyester laminating resins and to effectively integrate the body and the coating, thereby forming a unitary monolithic bathtub shell 11, by the final application of heat and (low) pressure to the stacked coating

and impregnated glass fibers to cure the polyesters therein.

In a second method of forming the instant bathtub shell 11 embodying the instant invention, which method shall be referred to hereinafter as method B, the first step is essentially the same as the first step of method A, as exemplified by Figure 4. In other words, the coating 24' is applied to a suitably formed mold form 25', suitably positioned on base members 26', in substantially the manner hereinbefore described. The resulting coated mold form 24' is thus shown as part of Figure 8.

Instead of employing sheets or glass fiber mats, however, a pre-formed body 23' is formed, in accordance with the showing of Figure 7. In such operation, glass fiber mats, strands or other bulk forms G are fed into a suitable shredder S through the hopper 31 and then through an output conduit 32 into a blower B which effectively blows the chopped glass fibers through a suitable nozzle and against a screen 33 which has been formed in substantially the shape of the ultimate glass fiber-resin impregnated body 23'. The air drives the airborne chopped-up glass fiber particles against the screen, so that the air may pass through and the fibers will be held against the screen in the position and thickness desired. This process affords the additional advantage of being able to readily provide extra thickness of glass fibers at specific locations in the body 23'. In general, the glass fiber raw material, whether mats, strands or the like, is not cut up by the shredder S into lengths that are shorter than about one or two inches, since it is desired to have the resulting unique cooperation between the elongated glass fibers and the hardened polyester hereinbefore described. After the glass fibers have been urged against the screen in the manner described, so as to form a glass fiber matting of substantially the shape and thickness ultimately desired in the body 23', a portion or all of the unsaturated polyester resin ultimately to be incorporated in the body 23' is sprayed upon or otherwise added to the glass fibers so as to impregnate the same, and preferably a short preliminary cure of the polyester is effected before the screen is separated from the preformed body 23'. In any event, the resin and the glass fibers are caused to cooperate to the extent that they will hold together as a cohesive unit 45 the body 23 formed within the screen 33. The screen 33 is then removed and the preformed body 23' is then positioned above the coating covered mold form 25' and slipped thereover so as to substantially fit the same. Next, an upper mold form 34, which has an inside cavity or base that has substantially the shape desired for the outside surface of the ultimately molded bathtub shell 11, and the top mold form 34 is then brought down against the back of the suitably positioned body 23', so as to urge the body 23' and the coating 24' against the mirror finished mold form 25'. By the use of the instant "matched metal die" method B, it is possible to obtain substantially better control of the exact thickness of the various portions of the bathtub shell 11, and also it is possible to effect a substantially greater molding pressure thereby permitting the use of slightly lower molding temperatures. By the use of high molding pressures, it is also possible to more effectively complete the polymerization of the polyesters in the stacked assembly, particularly if such polyesters have previously undergone a special cure, either for the purpose of causing the coating 24' to adhere more uniformly to the mold form 25' or for the purpose of integrating or holding together the body 23 prior to removing the same from the screen 33.

It will be appreciated that modification may be made in the instant structure, composition and method without departing from the scope of the instant invention.

We claim as our invention:

1. As an article of manufacture, a light weight bathtub having a suitably formed integral body of a laminate composed of one part of glass fibers embedded in two parts of normally rigid thermoset unsaturated polyester laminating resin, and having a smooth-surfaced glossy coating integrally formed upon the body, said coating consisting essentially of one part of pigment-size filler embedded in two parts of a thermoset unsaturated polyester mixture of equal parts of normally rigid and normally flexible polyesters.

2. As an article of manufacture, a light weight bathtub having a suitably formed integral body of a laminate

composed of one part of superimposed glass fiber mats, each substantially co-extensive with the body, embedded in two parts of normally rigid thermoset unsaturated polyester laminating resin, and having a smooth-surfaced glossy coating integrally formed upon the body, said coating consisting essentially of one part of finely ground amorphous silica filler, two parts of titanium dioxide pigment and six to seven parts of a thermoset unsaturated polyester mixture of 30-50% normally flexible polyester and 70-50% normally rigid polyester.

3. As an article of manufacture, a light weight bathtub having a suitably formed integral body of a 0.06-0.08 inch thick laminate composed of one part of glass fibers embedded in two parts of normally rigid thermoset unsaturated polyester laminating resin, and having a smooth-surfaced glossy coating integrally formed upon the body and having 0.01-0.02 inch thickness, said coating consisting essentially of one part of pigment-size filler embedded in two parts of a thermoset unsaturated polyester mixture of equal parts of normally rigid and normally flexible polyesters.

4. As an article of manufacture, a light weight bathtub having a suitably formed integral body of a laminate composed of one part of glass fibers embedded in two parts of normally rigid thermoset unsaturated polyester laminating resin, and having a smooth-surfaced glossy coating integrally formed upon the body and having 0.01-0.02 inch thickness, said coating consisting essentially of one part of finely ground amorphous silica filler, two parts of titanium dioxide pigment and six to seven parts of a thermoset unsaturated polyester mixture of 30-50% normally flexible polyester and 70-50% normally rigid polyester.

5. As an article of manufacture, a light weight bathtub having a suitably formed integral body 0.06-0.08 inch thick composed of one part of glass fibers embedded in two parts of normally rigid thermoset unsaturated polyester laminating resin, and having a smooth-surfaced glossy coating integrally formed upon the body and having 0.01-0.02 inch thickness, said coating consisting essentially of one part of finely ground amorphous silica filler, two parts of titanium dioxide pigment and six to seven parts of a thermoset unsaturated polyester mixture of 30-50% normally flexible polyester and 70-50% normally rigid polyester.

6. As an article of manufacture, a light weight bathtub having a suitably formed integral body of a laminate composed of one part of glass fibers embedded in one to three parts of normally rigid thermoset unsaturated polyester laminating resin, and having a smooth-surfaced glossy coating integrally formed upon the body, said coating consisting essentially of 10-30% titanium dioxide pigment, 5-15% finely ground amorphous silica filler and 60-70% of a cured polyester mixture of 50-60% unsaturated polyester and 40-50% saturated polyester.

7. A method of forming a light weight bathtub, that comprises applying a 0.01-0.02 inch coating to a mirror-finish convex surface of the contour of the inside of the bathtub, said coating being composed of 10-30% titanium dioxide pigment, 5-15% finely ground amorphous silica filler, a catalyst mixture of a metal drier and a ketone peroxide, and 60-70% of a polymerizable polyester mixture of 50-60% unsaturated polyester and 40-50% saturated polyester; then covering the coating with a layer of glass fibers impregnated with twice their weight of polymerizable unsaturated polyester containing a metal drier-ketone peroxide catalyst mixture; and finally applying heat and pressure to the coating and impregnated glass fibers to cure the polyesters therein.

8. A method of forming a light weight bathtub, that comprises applying a 0.01-0.02 inch coating to a mirror-finish convex surface of the contour of the inside of the bathtub, said coating being composed of 10-30% titanium dioxide pigment, 5-15% finely ground amorphous silica filler, a catalyst mixture of a metal drier and a ketone peroxide, and 60-70% of a polymerizable polyester mixture of 50-60% unsaturated polyester and 40-50% saturated polyester; then covering the coating with a plurality of plies of glass fiber mats each substantially coextensive with the convex surface and each impregnated with from one to three times their weight of polymerizable unsaturated polyester containing metal drier-ketone peroxide catalyst mixture; and finally

applying heat and pressure to the coating and impregnated glass fibers to cure the polyesters therein.

9. A method of forming a light weight bathtub, that comprises applying a 0.01-0.02 inch coating to a mirror-finish convex surface of the contour of the inside of the bathtub, said coating being composed of 10-30% titanium dioxide pigment, 5-15% finely ground amorphous silica filler, a catalyst mixture of a metal drier and a ketone peroxide, and 60-70% of a polymerizable polyester mixture of 50-60% unsaturated polyester and 40-50% saturated polyester; then placing upon the coating a pre-formed body of suitable size and shape of glass fibers impregnated with and bound together by one to three times their weight of partially cured unsaturated polyester; and finally clamping the body against the coating and applying heat to completely polymerize the polyesters and integrate the coating and body.

10. A method of forming a light weight bathtub, that comprises applying a thin coating to a mirror-finish convex surface of the contour of the inside of the bathtub, said coating being composed of one part of pigment-size white filler admixed with two parts of a polymerizable 50:50 mixture of saturated and unsaturated polyesters; then covering the coating with a layer of glass fibers impregnated with twice their weight of polymerizable unsaturated polyester containing a metal drier-ketone peroxide catalyst mixture; and finally applying heat and pressure to the coating and impregnated glass fibers to cure the polyesters therein.

15

5

10

11. A method of forming a light weight bathtub, that comprises applying a thin coating to a mirror-finish convex surface of the contour of the inside of the bathtub, said coating being composed of one part of finely ground amorphous silica filler, two parts of titanium dioxide pigment and six to seven parts of a polymerizable mixture of 30-50% saturated and 70-50% unsaturated polyesters; then covering the coating with a layer of glass fibers impregnated with twice their weight of polymerizable unsaturated polyester containing a metal drier-ketone peroxide catalyst mixture; and finally applying heat and pressure to the coating and impregnated glass fibers to cure the polyesters therein.

25

## References Cited in the file of this patent

## UNITED STATES PATENTS

| Number    | Name         | Date          |
|-----------|--------------|---------------|
| 2,478,165 | Collins      | Aug. 2, 1949  |
| 2,489,985 | Speight, Jr. | Nov. 29, 1949 |
| 2,495,640 | Muskat       | Jan. 24, 1950 |
| 2,614,058 | Francis      | Oct. 14, 1952 |
| 2,617,126 | Nebesar      | Nov. 11, 1952 |

## OTHER REFERENCES

Modern Plastics, March 1951, pages 55-59, 146, 149, 152, 155, 156, "The Promise of Reinforced Plastics in Defense."